

## UNITED STATES PATENT OFFICE

2,100,179

METHOD OF COATING METAL ARTICLES  
WITH ZINC

Allan Heathcote Williams, Chester, England

No Drawing. Application March 16, 1937, Serial No. 131,183. In Great Britain August 9, 1935

1 Claim. (Cl. 91—20.2)

This invention relates to an improved method of and means for coating metal articles with zinc, and has for its chief object to provide an improved process by means of which metal window frames may be very effectively and efficiently galvanized although, as will be appreciated from the following description, the present invention is by no means limited to a process for galvanizing metal window frames but is also applicable to the galvanizing of other metal articles.

The process of galvanizing a metal article according to the present invention is characterized in that the article to be galvanized is first given a coating of zinc by immersion in a bath of molten zinc, which coating is then heated out of contact with oxygen, or other gas or substance likely to have an injurious effect on the coating, for such a time and to such a temperature that the coating forms an alloy with the metal to be coated and is finally whilst still hot immersed in molten zinc, without contact with oxygen or other injurious gas or substance, whereby a coating of zinc firmly adhering to the previously produced alloy is obtained.

25 The apparatus for carrying out the present invention conveniently consists of a bath, the major portion of which is filled with molten lead or some other suitable substance of higher specific gravity than spelter, a comparatively thin layer 30 of molten spelter floating on top of the lead or the like. The articles to be coated are passed through the spelter into the molten lead where they are allowed to remain until they acquire the requisite temperature to enable the zinc to 35 form an alloy with the surface of the metal. The articles are then withdrawn through the layer of spelter where they receive a further coating of zinc.

The bath is preferably narrower at the bottom than at the top and has the heat applied to the sides of the same so that the heat lost on immersion of an article may be quickly made up.

40 When molten spelter is heated to a sufficiently high temperature to enable it to form an alloy with the article to be coated, it tends to attack the iron walls of the spelter bath and so rapidly increases the formation of dross and consequent 45 wastage of spelter. To a very large extent this disadvantage is overcome in the apparatus according to the present invention due to the relatively thin layer of zinc employed but, if desired, the spelter may be contained in a relatively shallow 50 retaining frame having its walls partly im-

mersed in the lead and having a clearance from the sides of the tank.

Describing now by way of example one convenient method of, and apparatus for, carrying out the present invention as applied to the galvanizing of window frames, the apparatus comprises a galvanizing bath which is of any convenient length and which is approximately two feet wide at the top at its widest part. The bath is about seven feet deep and tapers downwardly so that it is only about one foot wide at the bottom. By this means the heat of the furnace which is arranged on the sides of the bath is distributed over a wide area of the bath (which is conveniently made of iron) and so the heat lost on the immersion of the article to be galvanized into the bath can be quickly made up.

The bath is filled to the extent of about nine-tenths of its depth, viz., about six feet four inches, with molten lead or other suitable metal and on top of this molten lead or the like floats a layer of about eight or ten inches of molten zinc.

In use the window frame, or other article to be galvanized is, after being suitably "pickled" in the usual way, passed quickly through the thin upper layer of molten zinc into the molten lead beneath the same. The article is then allowed to remain in the molten lead until it acquires the same temperature or approximately the same temperature as the molten lead which is conveniently heated to about 550-570° C. During this time and when the article attains a temperature of about 490° C. the pores of the metal article seem to open and the preliminary coating of zinc which the article has received due to its initial passage through the molten zinc appears to form an alloy with the iron of the article to be galvanized.

When the article has attained the desired temperature it is withdrawn from the bath, passing again through the thin layer of zinc at the top of the bath. A skin-bond is formed through the zinc entering into the pores of the iron of the article to be galvanized and the coating is much more firmly attached than with the ordinary process of hot zinc galvanizing as carried out at the present time. For example, with the ordinary process carried out at the present time, the coating can be brushed off without much difficulty but this is impossible with articles galvanized by the process according to the present invention.

As above stated, the molten spelter may, if desired, be contained within a retaining frame

which will prevent it coming into contact with the sides of the bath.

The invention is capable of general application for zinc coating articles, but is particularly intended for forming a zinc coating on metal window frames which are very liable to rust.

I claim:—

A method of coating metal articles and more particularly window frames with zinc carried out 10 in a bath comprising a thin layer of molten zinc

floating on a body of molten lead, which method comprises heating the molten lead to a temperature of about 550° to 570° C., passing the article to be coated completely through the thin layer of molten zinc into the molten lead, leaving the article in the molten lead for a sufficient length of time to heat it to about 490° C., and finally withdrawing the heated article through the thin layer of molten zinc.

ALLAN HEATHCOTE WILLIAMS. 10